# EUROPEAN PATENT SPECIFICATION

(11) **EP 1 216 288 B1**
(45) Date of publication and mention of the grant of the patent: **16.04.2003**
(21) Application number: 00960644.3
(22) Date of filing: 07.09.2000
(51) Int. Cl.: C10L 1/18, C10L 10/04

(54) **FUEL COMPOSITION**
BRENNSTOFFZUSAMMENSETZUNG
COMPOSITION DE CARBURANT

(30) Priority: 10.09.1999 EP 99117853
(43) Date of publication of application: 26.06.2002
(73) Proprietor: OLEON, 9940 Ertvelde (BE)
(72) Inventor: PACKET, Dirk, B-1703 Asse (BE)
(74) Representative: Luys, Marie-José A.H.
(86) International application number: EP0008869
(87) International publication number: WO01019941

(56) References cited:
- EP-A- 0 773 278
- EP-A- 0 826 765
- WO-A-97/04044
- WO-A-98/11178
- WO-A-98/21293
- DE-A- 19 614 722
- FR-A- 1 405 551
- FR-A- 2 772 783
- US-A- 3 672 854
- US-A- 5 378 249

## Description

### FIELD OF THE INVENTION

The present invention relates to a fuel oil composition comprising a diesel fuel oil, and a fuel oil lubricity improver having improved cold storability. The invention further relates to the use of a composition having improved cold storability as a diesel fuel oil lubricity improver.

### BACKGROUND TO THE INVENTION AND PRIOR ART DISCUSSION

Various ester additives are known for addition to hydrocarbon compositions for various purposes. For example, US 2993773 describes esters of alkenyl succinic acid with a large variety of different alcohols. These esters are used to inhibit or prevent deposit-forming in hydrocarbon fuels. GB 1065398 describes how the lubricity of aviation turbojet fuels might be improved using partial esters of a number of different polyhydric alcohols, especially an ester of a C36 dimer acid and sorbitan monooleate. GB 1047493 is concerned with the addition of a lubricity additive to a lubricating oil in which the lubricity additive is a partial or mono ester of a dicarboxylic acid and an oil insoluble glycol such as the monoester of the C36 linoleic dimer acid and glycol.

WO 98/11178 discloses a polyol ester distillate fuel additive which exhibits improved lubricity, wear and frictional performance. The polyol ester has unconverted hydroxyl groups. Pentaerythritol is mentioned as one of the alcohol that can be used.

DE 196 14 722 A relates to additives for fuels and lubricants essentially consisting of a fatty acid mono-ester, or a mixture of mono- and di-esters of unsaturated fatty acids having 16-22 C atoms with at least two different polyols. These additives are said to exhibit better low temperature behaviour than corresponding monoesters or mono and diester of uniform polyols.

EP 0 826 765 A relates to fuel additives for improving lubricity. The additives comprise at least one partial ester of at least one monocarboxylic acid and at least one polyol. The monocarboxylic acid comprises a C4-C24 linear or branched, saturated or unsaturated acid that may be hydroxylated.

FR 2 772 783 relates to a lubricious additive for fuels having a low sulphur content (less than 500 ppm). The additive comprises a mixture of a glycerol monoester (5-95 wt.%) with another ester or an amine.

WO 98/21293 relates to low sulphur diesel fuels containing additives which increase lubricity and reduce smoke in the exhaust. The additive comprises a mixture of two different esters. A preferred ester is one which has no free hydroxyl groups.

WO 97/04044 relates to additives for improving the lubricity of fuel oils such as diesel fuel oil. This additive is a mixture of esters of unsaturated monocarboxylic acids. Preferred polyols for forming the esters are saturated aliphatic straight chain polyols.

US 3 672 854 relates to a middle distillate having an improved pour point, containing a pour point depressant. The depressant comprises an ester of a saturated C14-C26 carboxylic acid and a polyhydric alcohol having from 4 to 8 hydroxyl groups.

US 5 378 249 relates to a biodegradable two cycle engine oil composition comprising a heavy ester a light ester and additives. The oil is mixed with gasoline for the purpose of lubrication.

Diesel fuel oils generally comprise petroleum middle distillate fuel oils which boil within the range of 100°C to 400°C. There has recently been a drive to reduce the sulphur content of such diesel fuels so as to reduce sulphur dioxide emissions for environmental reasons. As of October 1996, the EU imposed a maximum sulphur content for diesel fuel oil of 0.05% by weight. As a result of this, a problem has arisen in that preparation of low sulphur content fuel oils also reduces the content in the fuels of other components such as polyaromatics. The problem is that the lubricity of the fuel is reduced and this can lead to engine failure. In order to overcome this problem, it has been proposed in WO 94/17160 to provide diesel fuel oil compositions with a lubricity improver additive. Particular examples of such an additive disclosed in WO 94/17160 are glycerol monooleate esters and di-isodecyl adipate esters. Glycerol monooleate esters are in commercial use as diesel fuel oil additives to enhance the lubricity of the diesel fuel oils. EP-A-0773278 also addresses this problem, providing as a lubricity improver additive a hydroxy-substituted carboxylic acid or acid derivative such as ricinoleic acid or glycerol monoricinoleate.

### SUMMARY OF THE INVENTION

The present invention is concerned with a new problem which arises with diesel fuel oil lubricity improvers such as glycerol monooleate. When lubricity improvers of this type are sold, manufacturers recommend that the product be stored above 10°C. This is necessary because, at lower temperatures, the known diesel fuel oil lubricity improvers become unstable with a tendency to cloud or even freeze. The requirement to store at above 10°C to prevent these drawbacks is inconvenient and costly for customers who have to provide specialised storage facilities. Thus, a further aim of the present invention is to provide a lubricity improver which also has improved cold storability.

The present invention aims to overcome the drawbacks of the prior art.

In a first aspect, the present invention provides use of a composition comprising a diester of a monocarboxylic acid and a polyhydric alcohol as a diesel fuel oil lubricity improver, wherein the monocarboxylic acid comprises a C₈-C₂₄ linear or branched chain unsaturated acid or a mixture thereof, and the polyhydric alcohol comprises an alcohol of the general formula:
CR¹R²R³R⁴, or a dimer, trimer or tetramer of the alcohol which is obtainable by condensation thereof, wherein
R¹, R² and R³ are each independently a C₁-C₁₂ linear or branched chain alkylol and R⁴ is a linear or branched chain C₁-C₁₂ alkyl or a linear or branched chain C₁-C₁₂ alkylol,
wherein the diester comprises at least two free hydroxyl groups.

In a second aspect, the present invention provides a fuel oil composition comprising a diesel fuel oil having a sulphur content of no more than 0.05% by weight and a fuel oil lubricity improver comprising a diester of a monocarboxylic acid and a polyhydric alcohol, wherein the monocarboxylic acid comprises a C₈-C₂₄ linear or branched chain unsaturated acid or a mixture thereof, and the polyhydric alcohol comprises an alcohol of the general formula:
CR¹R²R³R⁴, or a dimer, trimer or tetramer of the alcohol which is obtainable by condensation thereof wherein
R¹, R² and R³ are each independently a C₁-C₁₂ linear or branched chain alkylol and R⁴ is a linear or branched chain C₁-C₁₂ alkyl or a linear or branched chain C₁-C₁₂ alkylol,
wherein the diester comprises at least two free hydroxyl groups.

### DETAILED DESCRIPTION OF THE INVENTION

It is surprisingly found that, using the diesters of the present invention as a diesel fuel oil lubricity improver enables the product to be storable as a liquid at a temperature below 20°C, even at a temperature below -10°C. In addition to these cold stability properties, the diesters of the present invention possess ability comparable to the products currently on the market to improve the lubricity of diesel fuel oils. Accordingly, the need to use specialist storage facilities for the lubricity improvers is obviated.

The diester of the present invention may be part of a mixture optionally including higher esters such as a triester and a tetraester. R¹, R² and R³ are preferably each independently a C₁-C₄ linear or branched chain alkylol, more preferably CH₂OH. R⁴ is preferably a C₁-C₄ linear or branched chain alkyl or alkylol, such as CH₃, CH₂OH or CH₂CH₃. More preferably R⁴ is an alkylol so as to increase the number of free -OH groups in the diester. A particularly preferred alcohol component of the diester is pentaerythritol, although other alcohols such as trimethylolpropane (TMP) and trimethylolethane (TME) may be used. In any event, the final diester should have at least two free -OH groups. The lubricity improver used in the present invention may comprise a single pure diester, or may comprise a mixture containing two or more diesters.

The carboxylic acid component of the diester may be a linear or branched chain carboxylic acid which is unsaturated and is preferably a C₁₂-C₂₂ monocarboxylic acid. Typically, the carboxylic acid has an iodine value of 40 to 180, preferably an iodine value above 60, more preferably above 70, as measured in accordance with the AOCS (American Oil Chemists Society) Official Method cd-1-25. It is preferred to use an unsaturated carboxylic acid, since these are readily available and are often naturally-occurring. Particularly useful unsaturated carboxylic acids include oleic acid, linoleic acid, linolenic acid, palmitoleic acid, gadoleic acid, erucic acid and other unsaturated acids with 22 carbon atoms and mixtures thereof. The unsaturated carboxylic acid component may be selected from tall oil fatty acids, soybean fatty acids, rape seed fatty acids, sunflower seed fatty acids, fish oil and fatty acids, and cold fractionated tallow and palm oil fatty acids. The monocarboxylic acid may be substituted, for example, by at least one hydroxyl group. A suitable substituted monocarboxylic acid is ricinoleic acid.

In contrast with monoglycerides, the diesters of the present invention such as the pentaerythritol esters, have a cold stability which is independent of the molar ratio of fatty acid to alcohol. Thus, lubricity efficiency increases with a decrease in ratio of fatty acid to alcohol in both pentaerythritol and monoglycerides; in the monoglycerides the cold stability decreases whereas in the pentaerythritol diesters it does not.

Typically, in accordance with the present invention, the amount of fuel oil lubricity improver used in the fuel oil is in the range 1 to 1000ppm, preferably in the range 10 to 500ppm, most preferably in the range 10 to 200ppm.

The diester of the present invention may be used as the diesel fuel oil lubricity improver in pure form or in mixture with other components such as the conventional diesel fuel oil lubricity improvers, such as glycerol monooleate. Typically, the amount of diester of the present invention in such a mixture is in the range 60 to 100%wt, preferably in the range 80 to 100%wt, most preferably in the range 90 to 95%wt, especially around 92%. The properties of these mixtures are also improved over known lubricity improvers.

The present invention will now be described in further detail, by way of example only, with reference to the following Examples.

### EXAMPLES

### Example 1 - lubricity performance

All tests were done with the unadditized reference diesel fuel RF73-T-93, with a sulphur content of 0.05%.

The fuel oil incorporated an amount of lubricity improver as set out in Table 1 below so as to compare the effectiveness of lubricity improvers according to the present invention with those of the prior art. A High Frequency Reciprocating Rig (HFRR) test was carried out as described in D. Wei and H. Spikes, Wear, Vol. 111, No. 2, p. 217, 1986; and R. Caprotti, C. Bovington, W. Fowler and M. Taylor SAE paper 922183; SAE fuels and lubes. Meeting Oct. 1992; San Francisco, USA. The present applicants are aiming for a wear scar diameter of less than 400 microns at a dosage level of 100ppm.

**Table 1**

| *x wear scar diameter in micron for additized RF73-T-93* | | | |
|---|---|---|---|
| Dosage level /ppm | Glycerolmonooleate (comparative) | A | B |
| 0 | 552 | 552 | 552 |
| 100 | 305 | 328 | 381 |
| 200 | 315 | 328 | n.a. |

Lubricity improver A is a mixture of pentaerytritolmonooleate, pentaerytritoldioleate and pentaerytritoltrioleate including 39% diester. The olefin fraction used for the synthesis of this pentaerythritol ester and for the glycerolmonooleate was obtained by a cold fractionation of tallow fatty acids and has cloud point between 0°C and 6°C. Lubricity improver B is a mixture of 92% of A and 8% of the glycerolmonooleate.

### Example 2 - cold stability

The cold stability of both esters of example 1 was compared by measuring the cloud point according to ASTM method D5950 and the pour point according to ASTM method D5771. In addition, the cold stability of the best performing additive described in WO 97/04044 (additive A) was measured in the same way.

Additive A from WO 97/04044 was prepared by esterification of a commercial mixture of oleic and linoleic acids with glycerol to produce a mixed ester product comprising glycerol monooleate and glycerol monolinoleate in approximately equal proportions by weight, and containing minor amounts of glycerol di- and trioleate and linoleate. The results are presented in Table 2.

**Table 2**

| *cloud point and pour point of glycerolmonooleate and lubricity improvers A and B* | | | | |
|---|---|---|---|---|
| | Glycerolmonooleate (comparative) | Additive A from WO 97/04044 | A | B |
| Cloud point | +10°C | +1°C | -15°C | -14°C |
| Pour point | +3°C | -15°C | -27°C | -30°C |

The results show that both cloud point and pour point values are significantly lower in the pentaerythritol esters than in the prior art glycerolmonooleate and additive A.

### Example 3 - lubricity performance

As example 1, but the monoglyceride and the lubricity improver A were synthesized with tall oil fatty acids. Tall oil fatty acids as such are also included as comparative example. The results are shown in Table 3.

**Table 3**

| Dosage level /ppm | monoglyceride of tall oil fatty acids (comparative) | Tall oil fatty acids | A |
|---|---|---|---|
| 0 | 552 | 552 | 552 |
| 50 | 507 | n.a. | 493 |
| 100 | 336 | 339 | 318 |
| 200 | n.a. | n.a. | 310 |

### Example 4 - cold stability

The pour points of the different compounds mentioned in example 3 are compared. In addition to these compounds, the pour points of two additives described in WO 97/38965 are also compared. These additives are mixtures of trimethylolpropane monotalloate (TMP) (ester B of WO 97/38965) and glycerol monotalloate (ester A of WO 97/38965). In the context of this prior art disclosure, talloate means formed with tall oil fatty acids. The results are shown in Table 4.

**Table 4**

| Additive | Pour point (°C) |
|---|---|
| monoglyceride of tall oil fatty acids (comparative) | -27 |
| 30 mole% TMP ester B (comparative) | -36 |
| 50 mole% TMP ester B (comparative) | -33 |
| Tall oil fatty acids (comparative) | -12 |
| A | -51 |

Taken together, these results confirm that the esters of the present invention have good lubricity improvement properties for diesel fuel oils and superior cold storage properties as compared with the lubricity improvers of the prior art.

## Claims

1. Use of a composition comprising a diester of a monocarboxylic acid and a polyhydric alcohol as a diesel fuel oil lubricity improver, wherein the monocarboxylic acid comprises a C₈-C₂₄ linear or branched chain unsaturated acid or a mixture thereof, and the polyhydric alcohol comprises an alcohol of the general formula:
CR¹R²R³R⁴, or a dimer, trimer or tetramer of the alcohol which is obtainable by condensation thereof, wherein
R¹, R² and R³ are each independently a C₁-C₁₂ linear or branched chain alkylol and R⁴ is a linear or branched chain C₁-C₁₂ alkyl or a linear or branched chain C₁-C₁₂ alkylol
wherein the diester comprises at least two free hydroxyl groups.

2. Use according to claim 1, wherein R¹, R² and R³ are each independently a C₁-C₄ linear or branched chain alkylol.

3. Use according to claim 2, wherein R¹ and R² and R³ are each CH₂OH.

4. Use according to any one of claims 1-3, wherein R⁴ is a C₁-C₄ linear or branched chain alkyl or alkylol.

5. Use according to claim 4, wherein R⁴ is CH₃, CH₂OH or CH₂CH₃.

6. Use according to claim 4, wherein R⁴ is an alkylol.

7. Use according to any one of the preceding claims, wherein the alcohol comprises pentaerythritol.

8. Use according to any one of the preceding claims, wherein the monocarboxylic acid is substituted with at least one hydroxyl group.

9. Use according to any one of the preceding claims, wherein the monocarboxylic acid is a C₁₂-C₂₂ monocarboxylic acid.

10. Use according to any one of the preceding claims, wherein the carboxylic acid has an iodine value of 40-180, as measured in accordance with AOCS Official Method Cd-1-25.

11. Use according to any preceding claim, wherein the unsaturated carboxylic acid comprises a natural fatty acid.

12. Use according to claim 11, wherein the unsaturated carboxylic acid comprises oleic acid, linoleic acid, linolenic acid, palmitoleic acid, arachidic acid or mixtures thereof.

13. A fuel oil composition comprising a diesel fuel oil having a sulphur content of no more than 0.05% by weight and a fuel oil lubricity improver comprising a diester of a monocarboxylic acid and a polyhydric alcohol, wherein the monocarboxylic acid comprises a C₈-C₂₄ linear or branched chain unsaturated acid or a mixture thereof, and the polyhydric alcohol comprises an alcohol of the general formula:
CR¹R²R³R⁴, or a dimer, trimer or tetramer of the alcohol which is obtainable by condensation thereof wherein
R¹, R² and R³ are each independently a C₁-C₁₂ linear or branched chain alkylol and R⁴ is a linear or branched chain C₁-C₁₂ alkyl or a linear or branched chain C₁-C₁₂ alkylol,
wherein the diester comprises at least two free hydroxyl groups.

14. A fuel oil composition according to claim 13, wherein the diester is as defined in any one of claims 2 to 13.

15. A fuel oil composition according to claim 14, wherein the amount of the fuel oil lubricity improver in the fuel oil is in the range 10 to 500 ppm.

16. Use of a diester of a monocarboxylic acid and a polyhydric alcohol in a diesel fuel oil lubricity improver composition for improving the cold storability of the lubricity improver composition, wherein the monocarboxylic acid comprises a C₈-C₂₄ linear or branched chain unsaturated acid or a mixture thereof, and the polyhydric alcohol comprises an alcohol of the general formula:
CR¹R²R³R⁴, or a dimer, trimer or tetramer of the alcohol which is obtainable by condensation thereof, wherein
R¹, R² and R³ are each independently a C₁-C₁₂ linear or branched chain alkylol and R⁴ is a linear or branched chain C₁-C₁₂ alkyl or a linear or branched chain C₁₋C₁₂ alkylol
wherein the diester comprises at least two free hydroxyl groups.

## Patentansprüche

1. Verwendung einer Zusammensetzung, die einen Diester einer Monocarbonsäure und einen mehrwertigen Alkohol als Schmierfähigkeitsverbesserer für Dieselheizöl umfasst, wobei die Monocarbonsäure eine lineare oder verzweigtkettige ungesättigte C₈-C₂₄-Säure oder eine Mischung derselben umfasst und der mehrwertige Alkohol einen Alkohol der allgemeinen Formel:
CR¹R²R³R⁴ oder ein Dimer, Trimer oder Tetramer des Alkohols umfasst, das durch Kondensation desselben erhältlich ist, wobei
R¹, R² und R³ jeweils unabhängig ein lineares oder verzweigtkettiges C₁-C₁₂-Alkylol darstellen und R⁴ ein lineares oder verzweigtkettiges C₁-C₁₂-Alkyl oder ein lineares oder verzweigtkettiges C₁-C₁₂-Alkylol darstellt,
wobei der Diester mindestens zwei freie Hydroxylgruppen umfasst.

2. Verwendung nach Anspruch 1, wobei R¹, R² und R³ jeweils unabhängig ein lineares oder verzweigtkettiges C₁-C₄-Alkylol darstellen.

3. Verwendung nach Anspruch 2, wobei R¹ und R² und R³ jeweils CH₂OH darstellen.

4. Verwendung nach einem der Ansprüche 1 bis 3, wobei R⁴ ein lineares oder verzweigtkettiges C₁-C₄-Alkyl oder Alkylol darstellt.

5. Verwendung nach Anspruch 4, wobei R⁴ CH₃, CH₂OH oder CH₂CH₃ darstellt.

6. Verwendung nach Anspruch 4, wobei R⁴ ein Alkylol darstellt.

7. Verwendung nach einem der vorhergehenden Ansprüche, wobei der Alkohol Pentaerythrit umfasst.

8. Verwendung nach einem der vorhergehenden Ansprüche, wobei die Monocarbonsäure durch mindestens eine Hydroxylgruppe substituiert ist.

9. Verwendung nach einem der vorhergehenden Ansprüche, wobei die Monocarbonsäure eine C₁₂-C₂₂-Monocarbonsäaure ist.

10. Verwendung nach einem der vorhergehenden Ansprüche, wobei die Carbonsäure eine Iodzahl von 40 bis 180, der Offiziellen AOCS-Methode Cd-1-25 entsprechend gemessen, aufweist.

11. Verwendung nach einem der vorhergehenden Ansprüche, wobei die ungesättigte Carbonsäure eine natürliche Fettsäure umfasst.

12. Verwendung nach Anspruch 11, wobei die ungesättigte Carbonsäure Ölsäure, Linolsäure, Linolensäure, Palmitoleinsäure, Arachinsäure oder Mischungen derselben umfasst.

13. Heizölzusammensetzung, die Folgendes umfasst: ein Dieselheizöl mit einem Schwefelgehalt von nicht mehr als 0,05 Gew.% und einen Schmierfähigkeitsverbesserer für Heizöl, der einen Diester einer Monocarbonsäure und einen mehrwertigen Alkohol umfasst, wobei die Monocarbonsäure eine lineare oder verzweigtkettige ungesättigte C₈-C₂₄-Säure oder eine Mischung derselben umfasst und der mehrwertige Alkohol einen Alkohol der allgemeinen Formel:
CR¹R²R³R⁴ oder ein Dimer, Trimer oder Tetramer des Alkohols umfasst, das durch Kondensation desselben erhältlich ist, wobei
R¹, R² und R³ jeweils unabhängig ein lineares oder verzweigtkettiges C₁-C₁₂-Alkylol darstellen und R⁴ ein lineares oder verzweigtkettiges C₁-C₁₂-Alkyl oder ein lineares oder verzweigtkettiges C₁-C₁₂-Alkylol darstellt,
wobei der Diester mindestens zwei freie Hydroxylgruppen umfasst.

14. Heizölzusammensetzung nach Anspruch 13, wobei der Diester die in einem der Ansprüche 2 bis 13 angegebene Definition aufweist.

15. Heizöl nach Anspruch 14, wobei die Menge des Schmierfähigkeitsverbesserers für Heizöl in dem Heizöl im Bereich von 10 bis 500 ppm vorliegt.

16. Verwendung eines Diesters einer Monocarbonsäure und eines mehrwertigen Alkohols in einer Schmierfähigkeitsverbesserer-Zusammensetzung für Heizöl zum Verbessern der Kaltlagerfähigkeit der Schmierfähigkeitsverbesserer-Zusammensetzung, wobei die Monocarbonsäure eine lineare oder verzweigtkettige ungesättigte C₈-C₂₄-Säure oder eine Mischung derselben umfasst und der mehrwertige Alkohol einen Alkohol der allgemeinen Formel:
CR¹R²R³R⁴ oder ein Dimer, Trimer oder Tetramer des Alkohols umfasst, das durch Kondensation desselben erhältlich ist, wobei
R¹, R² und R³ jeweils unabhängig ein lineares oder verzweigtkettiges C₁-C₁₂-Alkylol und R⁴ ein lineares oder verzweigtkettiges C₁-C₁₂-Alkyl oder ein lineares oder verzweigtkettiges C₁-C₁₂-Alkylol darstellt,
wobei der Diester mindestens zwei freie Hydroxylgruppen umfasst.

## Revendications

1. Utilisation d'une composition contenant un diester d'acide monocarboxylique et un alcool polyvalent comme additif d'onctuosité pour un carburant diesel, où l'acide monocarboxylique comporte un acide insaturé en C₈ à C₂₄ à chaîne linéaire ou ramifiée, ou un mélange de tels acides, et l'alcool polyvalent comporte un alcool de la formule générale:
CR¹R²R³R⁴, ou un dimère, un trimère ou un tétramère de l'alcool que l'on peut obtenir par leur condensation, dans laquelle
R¹, R² et R³ représentent indépendamment les uns des autres un alcool alkylique en C₁ à C₁₂ à chaîne linéaire ou ramifiée et R⁴ est un radical alkyle en C₁ à C₁₂ à chaîne linéaire ou ramifiée ou un alcool alkylique en C₁ à C₁₂ à chaîne linéaire ou ramifiée,
où le diester comporte au moins deux groupes hydroxyle libres.

2. Utilisation selon la revendication 1, où R¹, R² et R³ représentent chacun indépendamment un alcool alkylique en C₁ à C₄ à chaîne linéaire ou ramifiée.

3. Utilisation selon la revendication 2, où R¹ et R² et R³ représentent chacun CH₂OH.

4. Utilisation selon l'une quelconque des revendications 1 à 3, où R⁴ est un radical alkyle ou un alcool alkylique en C₁ à C₄ à chaîne linéaire ou ramifiée.

5. Utilisation selon la revendication 4, où R⁴ représente CH₃, CH₂OH ou CH₂CH₃.

6. Utilisation selon la revendication 4, où R⁴ est un alcool alkylique.

7. Utilisation selon l'une quelconque des revendications qui précèdent, où l'alcool comprend du pentaérythritol.

8. Utilisation selon l'une quelconque des revendications qui précèdent, où l'acide monocarboxylique est substitué par au moins un groupe hydroxyle.

9. Utilisation selon l'une quelconque des revendications qui précèdent, où l'acide monocarboxylique est un acide monocarboxylique en C₁₂ à C₂₂.

10. Utilisation selon l'une quelconque des revendications qui précèdent, où l'acide carboxylique présente un indice d'iode de 40 à 180, mesuré par la méthode officielle Cd-1-25 de l'AOCS.

11. Utilisation selon l'une quelconque des revendications qui précèdent, où l'acide carboxylique insaturé comprend un acide gras naturel.

12. Utilisation selon la revendication 11, où l'acide carboxylique insaturé contient de l'acide oléique, de l'acide linoléique, de l'acide palmitoléique, de l'acide arachidique, ou leurs mélanges.

13. Composition de carburant comportant un carburant diesel présentant une teneur en soufre non supérieure à 0,05% en poids et contenant un additif d'onctuosité pour carburant comprenant un diester d'un acide monocarboxylique et d'un alcool polyvalent, où l'acide monocarboxylique comprend un acide insaturé en C₈ à C₂₄ à chaîne linéaire ou ramifiée, et l'alcool polyvalent comprend un alcool de la formule générale:
CR¹R²R³R⁴, ou un dimère, un trimère ou un tétramère de l'alcool que l'on peut obtenir par leur condensation, dans laquelle
R¹, R² et R³ représentent indépendamment les uns des autres un alcool alkylique en C₁ à C₁₂ à chaîne linéaire ou ramifiée et R⁴ est un radical alkyle en C₁ à C₁₂ à chaîne linéaire ou ramifiée ou un alcool alkylique en C₁ à C₁₂ à chaîne linéaire ou ramifiée
où le diester comporte au moins deux groupes hydroxyle libres.

14. Composition de carburant selon la revendication 13, où le diester est tel que défini dans l'une des revendications 2 à 13.

15. Composition de carburant selon la revendication 14, où la quantité de l'agent d'onctuosité pour carburant dans le carburant est de l'ordre de 10 à 500 ppm.

16. Utilisation d'un diester d'un acide monocarboxylique et d'un alcool polyvalent dans une composition d'agent d'onctuosité pour carburant diesel, aux fins d'amélioration de l'entreposage à froid de la composition d'agent d'onctuosité, où l'acide monocarboxylique comprend un acide insaturé en C₈ à C₂₄ à chaîne linéaire ou ramifiée, ou un mélange de tels acides, et l'alcool polyvalent comprend un alcool de la formule générale:
CR¹R²R³R⁴, ou un dimère, un trimère ou un tétramère de l'alcool que l'on peut obtenir par leur condensation, dans laquelle
R¹, R² et R³ représentent indépendamment les uns des autres un alcool alkylique en C₁ à C₁₂ à chaîne linéaire ou ramifiée et R⁴ est un radical alkyle en C₁ à C₁₂ à chaîne linéaire ou ramifiée ou un alcool alkylique en C₁ à C₁₂ à chaîne linéaire ou ramifiée,
où le diester comporte au moins deux groupes hydroxyle libres.
